

# United States Patent Office

2,705,184

Patented Mar. 29, 1955

1

2,705,184

## PROCESS FOR THE PRODUCTION OF RAYON PRODUCTS

Nicolas Drisch and Paul Herrbach, Paris, France, assignors to Textile & Chemical Research Company, Ltd., St. Peter Port, Guernsey, Channel Islands, a corporation of Great Britain

No Drawing. Application July 3, 1952,  
Serial No. 297,180

Claims priority, application France January 15, 1952

8 Claims. (Cl. 18—54)

This invention relates to the production of viscose rayon, artificial horse-hair, ribbons and the like and particularly to the production of viscose staple fibre.

In co-pending application No. 193,746, now Patent No. 2,607,955, there is described a process for spinning viscose having a viscosity of at least 400 poises and a  $\gamma$ -value above 60 into coagulating baths of low acid (e. g. sulphuric acid) concentration, the filamentary products being fixed by treatment with hot aqueous liquid.

The process described in the application has since been the subject of long research, the remarkable results of which form the subject of the present invention, which relates to a modified process by means of which it is possible to obtain fibres having a remarkably high resistance to repeated bending. The known processes for the production of rayon, including those described in the said co-pending application, do not enable fibres to be obtained which have as high a resistance to repeated bending as is desired. Resistance to bending is of fundamental importance to the behaviour of artificial staple fibres during use and the modified process of the present invention is therefore more particularly directed to the production of staple fibre.

It is an object of the present invention to provide artificial filamentary materials of viscose which have a remarkably high resistance to repeated bending. A further object of this invention is to provide artificial viscose staple fibre which has a high resistance to repeated bending. A still further object is to provide processes whereby such filamentary materials and staple fibre may be obtained. Another object of the invention is to provide a combination of a viscose spinning solution and a coagulating bath of such compositions that the aforesaid products are obtained. Other objects of the invention will appear hereinafter.

It has been discovered that products of very high resistance to bending can be obtained, in processes using viscose of the aforesaid special properties and dilute acid coagulating baths by increasing the sodium sulphate content of the coagulating bath. A content of sodium sulphate up to 25 g./litre in the coagulating bath is known, and results from the reaction between the caustic soda in the viscose and the weakly acid bath, taking into account the constant renewal of the bath.

It has now been discovered that the resistance to repeated bending increases substantially if the sodium sulphate content is increased to at least 50 grams per litre, and preferably to 80 to 150 grams per litre, the upper limit being imposed by the solubility of the sodium sulphate in the slightly acid bath.

2

As described in the co-pending application, it is essential to use cellulose pulp of very high degree of polymerisation, for example of at least 700 to 800, and to conduct the preparation of the viscose under conditions such that the cellulosic material is depolymerised to a minimum extent. It should, for the purposes of the present invention have a viscosity of at least 300 poises and a  $\gamma$ -value above 60 for satisfactory spinning. Its cellulose content may be 4-8% or more. The caustic soda content may vary, but is preferably 3-5%, although it may be higher.

The following examples will serve to illustrate the invention but are not to be regarded as limiting it in any way.

### EXAMPLE I

Linters of a degree of polymerisation of 700-800 are mixed in caustic soda (concentration 225-240 g./litre) and pressed until the ratio of the final weight of the alkali-cellulose to the weight of  $\gamma$ -cellulose contained in the pulp used is 2.8. The alkali-cellulose is not ripened but is shredded and then xanthogenated with 55% of carbon disulphide (calculated on the  $\gamma$ -cellulose content of the pulp) at between 25° and 30°. Degradation due to the action of atmospheric oxygen is limited to a minimum during the treatment, preferably by working under vacuum or in an inert atmosphere.

The cellulose xanthogenate is worked into a paste with concentrated caustic soda at -5 to +5° C. and the product is mixed with dilute caustic soda or water to produce a viscose containing 6% cellulose and 3% to 5% caustic soda. The viscose obtained is not aged. It has a  $\gamma$ -value above 70 and a viscosity of about 400 poises.

It may be mentioned here that viscoses of high degree of polymerisation having viscosities substantially lower than 300 poises do not spin satisfactorily.

The viscose is spun from a horizontal spinneret, the stream of fibres leaving the spinneret rising vertically in the spinning bath. A dilute sulphuric acid coagulating bath is employed which may contain up to 25 grams per litre of sulphuric acid at room temperature. The sodium sulphate content of the coagulating bath must be greater than 50 grams per litre, and preferably greater than 80 grams per litre. The gel obtained following the coagulation is subjected to a stretch which may vary between 30% and 150% according to the characteristics which it is desired to impart to the thread. The gel is then treated with boiling water to regenerate the cellulose.

Under these conditions, excellent spinning is achieved. The bundle of filaments is subjected to the usual finishing treatments and dried. It may be cut into lengths by means of a cutting machine before the regeneration treatment, or the finished bundle may be stretched continuously until it breaks for the purpose of directly forming a sliver.

The following table shows the results of tests applied to the staple thus obtained, as compared with staple obtained when employing baths containing less sodium sulphate. In the first three columns are indicated the results obtained with three fibres spun from baths containing about 30 grams per litre of sodium sulphate. In the last three columns are shown the results obtained with a fibre spun into a bath containing 50 grams/litre of sodium sulphate (fibre D), and with two fibres spun into baths containing 115 grams per litre of sodium sulphate. All the baths contain 30 g./litre of sulphuric acid.

Table

|                              | Fibre A<br>30 g./l.<br>Na <sub>2</sub> SO <sub>4</sub> | Fibre B<br>30 g./l.<br>Na <sub>2</sub> SO <sub>4</sub> | Fibre C<br>30 g./l.<br>Na <sub>2</sub> SO <sub>4</sub> | Fibre D<br>50 g./l.<br>Na <sub>2</sub> SO <sub>4</sub> | Fibre E<br>115 g./l.<br>Na <sub>2</sub> SO <sub>4</sub> | Fibre F<br>115 g./l.<br>Na <sub>2</sub> SO <sub>4</sub> |
|------------------------------|--------------------------------------------------------|--------------------------------------------------------|--------------------------------------------------------|--------------------------------------------------------|---------------------------------------------------------|---------------------------------------------------------|
| Mean count.....              | 1 D 49                                                 | 1 D 30                                                 | 1 D 49                                                 | 1 D 38                                                 | 2 D 37                                                  | 1 D 35                                                  |
| Percent irregularity.....    | 4.7                                                    | 7                                                      | 6.6                                                    |                                                        |                                                         |                                                         |
| Rkm, dry.....                | 36.2                                                   | 23.1                                                   | 28                                                     | 32.1                                                   | 31.3                                                    | 33.7                                                    |
| Rkm, wet.....                | 27                                                     | 19                                                     | 21.3                                                   | 25.6                                                   | 24.1                                                    | 27.3                                                    |
| Dry elongation, percent..... | 9.2                                                    | 7.8                                                    | 11.1                                                   | 10.5                                                   | 13.3                                                    | 11.7                                                    |
| Wet elongation, percent..... | 8.8                                                    | 7.3                                                    | 14.8                                                   | 11                                                     | 15.3                                                    | 13                                                      |
| Quality factor.....          | 80                                                     | 51                                                     | 82                                                     | 85                                                     | 93.5                                                    | 98.1                                                    |
| D. P.....                    | 583                                                    | 488                                                    | 496                                                    | 517                                                    | 610                                                     |                                                         |
| Dye affinity.....            | 10                                                     | 3                                                      | 25                                                     |                                                        | 18                                                      |                                                         |
| Resistance to bending.....   | 270                                                    | 566                                                    | 700                                                    | 870                                                    | 2,400                                                   | 6,620                                                   |

It is pointed out that "Rkm" is the "kilometric length," that is to say, the length of fibre of the same type which must be suspended from the fibre to be tested in order to break it, and represents nine times the tenacity.

The quality factor is the wet tenacity multiplied by the square root of the wet elongation. The D. P. is the mean degree of polymerisation. The resistance to bending is measured as the number of bends before break with a load of 0.33 g. per denier.

The remarkable increase in repeated bending obtained by means of baths containing large quantities of sodium sulphate will be seen.

#### EXAMPLE II

Viscose is prepared under approximately the same conditions as in Example I, with a cellulose content of 7% and a caustic soda content of 4%. The viscosity is 400 poises, the  $\gamma$  is 75 and the D. P. of the cellulose in the viscose is 410.

This viscose is spun at room temperature into a bath of sulphuric acid which may contain up to 30 grams of sulphuric acid per litre, and which contains in addition 30 grams of sodium sulphate per litre in one case, and 100 grams of sodium sulphate in another case, with the usual stretching of the gel, acid cutting and decomposition in boiling water followed by washing and finishing treatments under the usual known conditions.

The fibres of 1.5 d. obtained have similar serimetric characteristics namely:

|                |         |      |
|----------------|---------|------|
| Dry tenacity   | g./d.   | 3.4  |
| Wet tenacity   | g./d.   | 2.8  |
| Dry elongation | percent | 10.5 |
| Wet elongation | do      | 10.9 |

but in the first case it withstands 600 bending cycles, and in the second case 2000 bending cycles, the load being 0.33 g./d. as before.

These tests also confirm the very substantial improvement of the resistance to repeated bending due to the increase in the sodium sulphate content of the coagulating bath.

We claim:

1. Process for the production of viscose rayon suitable for the production of staple fibre which comprises spinning viscose prepared from cellulose pulp having a degree of polymerisation of 700 minimum, without ripening the alkali-cellulose and without ageing of the viscose, the viscose having a viscosity of at least 300 poises, and a gamma higher than 70, the coagulating bath employed comprising up to 25 grams/litre of sulphuric acid, and at least 50 grams per litre of sodium sulphate.

2. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 25 grams/litre of sulphuric acid, and at least 80 grams per litre of sodium sulphate.

3. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% to 5%, a viscosity of at least 300 poises, and a gamma higher than 70, the coagulating bath employed comprising up to 30 grams/litre of sulphuric acid, and at least 50 grams per litre of sodium sulphate, the viscose being spun vertically upwards from a horizontal spinneret.

4. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 30 grams/litre of sulphuric acid, and at least 50 grams per litre of sodium sulphate, and subjecting the spun filamentary products to high stretch continuously with their production.

5. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 30 grams/litre of sulphuric acid, and at least 50 grams per litre of sodium sulphate, and converting the spun filamentary products to staple fibre.

6. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 30 grams/litre of sulphuric acid, and at least 80 grams per litre of sodium sulphate, the viscose being spun vertically upwards from a horizontal spinneret.

7. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 30 grams/litre of sulphuric acid, and at least 50 grams per litre of sodium sulphate, the viscose being spun vertically upwards from a horizontal spinneret, and subjecting the spun filamentary products to high stretch continuously with their production.

8. Process for the production of viscose rayon suitable for the production of staple fibre which comprises spinning viscose prepared from cellulose pulp having a degree of polymerisation of 700 to 800, without ripening the alkali-cellulose and without ageing of the viscose, the viscose having a cellulose content of 4% to 8% and a caustic soda content of between 3% and 5%, a viscosity of at least 300 poises, and a gamma higher than 70, the coagulating bath employed comprising up to 30 grams/litre of sulphuric acid, and at least 50 grams per litre of sodium sulphate, and subjecting the spun filamentary products to high stretch continuously with their production, and converting the spun filamentary products to staple fibres.

#### References Cited in the file of this patent

#### UNITED STATES PATENTS

70 2,511,699 Drisch et al. \_\_\_\_\_ June 13, 1950  
2,607,955 Drisch et al. \_\_\_\_\_ Aug. 26, 1952

#### OTHER REFERENCES

"Latest Survey of New Synthetic Fibers," Rayon Textile  
75 Monthly, January 1945, page 64 (18).